

## UNITED STATES PATENT OFFICE

RENÉ CLAVEL, OF BASEL-AUGST, NEAR BASEL, SWITZERLAND

## TREATMENT OF CELLULOSE DERIVATIVES OF PRODUCTS MADE THEREWITH

No Drawing.

Application filed January 29, 1926. Serial No. 84,764.

This invention relates to the dyeing (under which term is included dyeing, printing or stencilling operations generally) of artificial filaments, threads, yarns, fabrics, films or other products made from or containing cellulose acetate, hereinafter referred to as cellulose acetate goods.

It is known that the affinity of dyestuffs for cellulose acetate can be improved by adding to the dyebath or the printing paste certain organic and inorganic compounds in the form of acids, salts or bases. The substances hitherto employed were such as to modify the surface of the fibre by hydrolysis or by a solvent or similar swelling action, so as to render the surface of the fibre capable of absorbing the dyestuff. Alternatively, substances were used which acted as dispersing agents, the dyestuffs being thus rendered capable of being more readily absorbed by the fibre.

Processes for treating cellulose acetate goods to increase their weight and volume, and for other purposes, are described in the U. S. A. patent application of Dr. Camille Dreyfus and Herbert Platt, No. 57,956, filed September 22, 1925, and U. S. Patent No. 1,731,298 of October 15, 1929.

Now as the result of much experiment it has been found that by loading cellulose acetate goods with tin phosphate or other metallic salt or salts that is or are insoluble in water, and particularly salts that act as loading agents for natural silk, the loaded goods display an increased affinity for dyestuffs colouring matters or colouring compounds, and can not only be dyed, printed or stencilled with the dyes, colouring matters or colouring compounds ordinarily used for dyeing and similarly treating cellulose acetate, all hereinafter referred to by the generic term dyestuffs, but are also capable of being satisfactorily dyed printed or stencilled with dyestuffs or colouring matters having only a feeble affinity or no affinity for cellulose acetate, such for example as dyestuffs contain-

ing sulphonic acid groups and the dyestuffs or colouring matters used for cotton goods.

According to this invention, goods made of or containing cellulose acetate are loaded with a metallic salt or salts that is or are insoluble in water, preferably such as act as loading agents for natural silk, and are afterwards dyed, printed or stencilled with dyestuffs, colouring matters or colouring compounds in any usual or suitable way.

The loading agents may be deposited on the goods by treatment in succession with a bath containing in solution a salt or salts of a metal or metals such as tin, zinc, tungsten, or aluminium and a bath containing a solution of phosphate, silicate, tannin or other compound or compounds adapted to deposit the metal or metals as an insoluble salt or salts upon the goods.

The first bath is preferably maintained at a temperature not lower than 50° C. during the treatment of the goods, but lower temperatures may also be used.

The loading operation may be repeated, it being found that with each successive loading operation the increase in the capacity of the goods for absorbing dyestuffs becomes greater and greater.

Cellulose acetate goods, after they have been loaded in this manner, may be dyed with direct, acid, basic and other dyestuffs.

The process presents a marked advantage over those heretofore in use in that the colouring of the goods is of greater depth and brilliancy.

For instance, using a bath containing 1 per cent. (calculated on the fibre) of Janus black D, Color Index No. 134, with a cellulose acetate fibre that had been loaded with 30 per cent. of tin phosphate, a deep black was obtained; while with untreated fibre a light grey was produced, and with a fibre subjected to superficial hydrolysis there resulted a medium grey. Using rhodamine G Color Index No. 750, under similar conditions, a cellulose

acetate fibre loaded with tin phosphate was dyed to a brilliant deep shade, in marked contrast to the paler shade obtained on unloaded fibre.

5 The colours produced in accordance with this invention may readily be discharged, the process thus presenting advantages over those hitherto in use.

10

*Example I*

15 1 kilo. of cellulose acetate yarn in hanks is worked for 1 hour in a bath containing 90 grams of tin (in the form of stannic chloride) per litre, the bath being maintained at a temperature of 50° C. The yarn is removed from the bath, washed twice with hard water, and centrifuged. The yarn is now placed in a bath containing 60 grams of disodium phosphate per litre. After treatment 20 in the bath for 1/2 hour at a temperature of 60° C. the yarn is removed and washed with soft water. The loaded yarn is then dyed in a bath containing 20 litres of water in which is dissolved 10 gms. of Janus black 25 D, Color Index No. 876, and 60 cc. of acetic acid, the bath being maintained at 60° C. The yarn is left in the bath for 1/2 hour and is then centrifuged and dried.

30

*Example II*

35 Cellulose acetate fabrics are loaded and prepared for printing by treatment in successive baths of stannic chloride and disodium phosphate in the manner described in Example I. If a heavier loading and an enhanced affinity for dyestuffs is desired, mono-sodium phosphate may be used in the second bath, or the loading operation may be repeated as often as desired or advisable. 40 Between each loading operation the goods are washed in an acid bath constituted by adding 60 cc. of hydrochloric acid of 20° Bé. to 20 litres of water.

45

The loaded fabric is printed with a painting paste consisting of—

|                                      |  |
|--------------------------------------|--|
| 50 grams of Capri blue               |  |
| 25 grams of concentrated acetic acid |  |
| 325 grams of water                   |  |
| 50 600 grams of a thick gum          |  |
| <hr/>                                |  |
| 1000                                 |  |

The printed goods are thoroughly dried and 55 steamed for about 1/2 hour and finally well washed and dried.

It will be understood that the process is not limited to the procedure set forth in the preceding examples, but may vary widely 60 therefrom without departing from the invention. The process, moreover, is applicable to the dyeing, printing or stencilling of mixed yarns, fabrics or materials containing filaments or yarns of cellulose acetate associated with other fibres or yarns, such as cotton or

other cellulose fibres (natural or artificial), wood, and silk, said mixed yarns, fabrics or materials being likewise included in the term cellulose acetate goods.

The term "loading" is employed in this specification in the ordinary technical significance in which it is employed in connection with natural silk, that is to say, to denote the technical operation of increasing the weight of the material under treatment; it does not include the production of such relatively small increases in weight as may be associated with processes of dyeing, such for example, as those effected with the aid of mordants.

70 75 What I claim and desire to secure by Letters Patent is:

1. A process of dyeing cellulose acetate materials which comprises loading said materials by forming therein a water insoluble metallic salt and thereafter dyeing the loaded materials with a dyestuff that has but little affinity for unloaded cellulose acetate material.

80 85 90 95 2. A process of dyeing cellulose acetate materials which comprises loading said materials by an operation comprising two stages, the first consisting in swelling and impregnating the materials with a solution of a salt of a loading metal, and the second consisting in treating the materials with a solution of a compound adapted to fix the metal therein as an insoluble salt, and thereafter dyeing the loaded materials with a dyestuff that has but little affinity for unloaded cellulose acetate material.

100 105 110 115 3. A process of dyeing cellulose acetate materials which comprises loading said materials by swelling and impregnating them with a solution of a salt of tin and then treating them with a solution of a compound adapted to fix the tin therein as an insoluble salt, and thereafter dyeing the loaded materials with a dyestuff that has but little affinity for unloaded cellulose acetate material.

120 125 130 4. A process of dyeing cellulose acetate materials which comprises loading said materials by swelling and impregnating them with a solution of stannic chloride and then treating them with a solution of a compound adapted to fix the tin therein as phosphate of tin, and thereafter dyeing the loaded materials in any suitable manner.

5. A process of dyeing cellulose acetate materials which comprises loading said materials by swelling and impregnating them with a solution of a salt of a loading metal and then treating them with a solution of a compound adapted to fix the metal therein as an insoluble phosphate, and thereafter dyeing the loaded materials in any suitable manner.

12 13 6. A process of dyeing cellulose acetate materials which comprises loading said materials by swelling and impregnating them

with a heated solution of a salt of a loading metal and then treating with a solution of a compound adapted to fix the metal therein as an insoluble salt and thereafter dyeing 5 the loaded materials with a dyestuff that has but little affinity for unloaded cellulose acetate material.

7. A process of dyeing cellulose acetate materials which comprises loading said materials by first swelling and impregnating them with a heated solution of a chloride of a loading metal and then treating them with a solution of a compound adapted to fix the metal therein as an insoluble salt, and there- 15 after dyeing the loaded materials with a dyestuff that has but little affinity for unloaded cellulose acetate material.

8. A process of dyeing cellulose acetate materials which comprises loading said materials by first swelling and impregnating them with a solution of a chloride of a loading metal at a temperature of about 50° C., and then treating them with a solution of a compound adapted to fix the metal therein as an insoluble salt, and thereafter dyeing the loaded materials with a dyestuff that has but little affinity for unloaded cellulose acetate material.

9. A process of dyeing cellulose acetate 30 materials which comprises loading said materials by first treating them with a heated solution of stannic chloride and then treating them with a solution of a compound adapted to fix the tin therein as an insoluble salt, and 35 thereafter dyeing the loaded materials with a dyestuff that has but little affinity for unloaded cellulose acetate material.

10. A process of dyeing cellulose acetate materials which comprises loading said materials by first treating them with a solution of stannic chloride at a temperature of about 40 50° C., and then treating them with a solution of a compound adapted to fix the tin therein as an insoluble salt, and thereafter dyeing the 45 loaded materials with a dyestuff that has but little affinity for unloaded cellulose acetate material.

11. A process of dyeing cellulose acetate materials which comprises loading said materials by swelling and impregnating them with a solution of stannic chloride and then treating them with a solution of a compound adapted to fix the tin therein as an insoluble salt, and thereafter dyeing the loaded materials with a dyestuff that has but little affinity for unloaded cellulose acetate material.

12. As a new article of manufacture, a material comprising cellulose acetate loaded 60 with a water-insoluble metal salt, and a dyestuff that has but little affinity for unloaded cellulose acetate yarn.

13. As a new article of manufacture, a material comprising cellulose acetate loaded 65 with a water-insoluble tin salt, and a dye-

stuff that has but little affinity for unloaded cellulose acetate yarn.

14. As a new article of manufacture, a material containing filaments comprising loaded cellulose acetate, and a dyestuff that has but 70 little affinity for unloaded cellulose acetate yarn.

15. As a new article of manufacture, a material containing filaments comprising cellulose acetate loaded with a water-insoluble 75 metal salt, and a dyestuff that has but little affinity for unloaded cellulose acetate yarn.

16. As a new article of manufacture, a fabric containing filaments comprising cellulose acetate loaded with a water-insoluble 80 metallic salt, said fabric having a pattern thereon printed with a dyestuff having but little affinity for unloaded cellulose acetate yarn.

17. A fabric containing loaded cellulose 85 acetate yarn dyed with a dyestuff that has but little affinity for unloaded cellulose acetate yarn.

In testimony whereof I have hereunto subscribed my name.

RENE CLAVEL.

95

100

105

110

115

120

125

130